

Patented June 18, 1929.

1,717,575

# UNITED STATES PATENT OFFICE.

EUGENE L. MESSLER, OF PITTSBURGH, PENNSYLVANIA.

## REFRACTORY COMPOSITION FOR HOT TOPS.

No Drawing. Original application filed December 8, 1926, Serial No. 153,250. Divided and this application filed September 17, 1927. Serial No. 220,288.

This invention relates to a composition for use in the manufacture of hot tops for ingot molds and the like, and constitutes a division of copending application Serial No. 5 153,250, filed December 8, 1926.

As is well known in the art, feeders or hot tops are manufactured of clay or some other more or less refractory composition, and are placed on the ingot mold prior to the operation 10 of teeming or pouring the ingot. These hot tops are used not only as a receptacle for the sink head of the ingot, but also serve to keep the metal in a fluid condition during pouring, so that it will feed properly into 15 the mold.

Certain problems are encountered in the manufacture and use of hot tops. One such problem is caused by the fragility of the material of which hot tops have been made, 20 which is apt to lead to their breakage in shipment. Another problem is that most hot tops during a preheating operation, or when they come into contact with metal during pouring are apt to crumble, slag, crack, or 25 spall. These actions are apt to result in the inclusion of particles of the hot top in the ingot. Another problem is due to the fact that a hot top during pouring may slag sufficiently to become attached to the sink head; 30 this possibility necessitating that a hot top be blocked up on the ingot mold, so that the blocking may be removed after the ingot has been teemed to permit the top to settle with the steel as it contracts.

As stated above, the general function of a hot top is to provide a good insulating reservoir to retain the heat of the metal, so that it will fit well into the mold. Previously a 35 thoroughly successful material for hot tops had not been evolved. If a hot top be of too dense a material, such as plastic clay, such material will be too good a conductor of heat to permit the hot top to perform its function satisfactorily. It is also so dense that it will 40 crack and spall badly giving brick inclusions in the steel. If, on the contrary, the hot top be made of relatively porous material such as slag, this material is not sufficiently bonded to prevent the scaling off of particles from 45 the body of the hot top.

The object of the present invention is to provide a composition for the manufacture of hot tops of such nature that the hot tops made thereof will not be readily broken during 50 shipment, or when placed in position on

the ingot mold; and which gives the hot top high insulating qualities, without crumbling, slagging, or cracking, or spalling when subjected to applied heat or to contact with the molten metal.

A top made of the special composition of the present invention has the advantages of a relatively high fusing point, relatively low conductivity of heat, and sufficient strength to avoid breakage of the hot top during shipment and use. Such desirable composition comprises flint clay, grog (granulated or powdered brick) and plastic clay. The proportions of these ingredients may be varied within fairly wide limits in accordance with the temperature to which the hot top is to be subjected, and in accordance with the probable shocks which it must withstand during shipment and use. A desirable composition may be secured by utilizing the grog 60 in the proportion of 10% to 20% of the total composition, flint clay in the proportion of 40% to 60% of the total composition and plastic clay as the remaining ingredient. A composition comprising the constituents in 65 such proportions as to be applicable to a wide general use comprises 10% of grog, 45% of flint clay, and 45% of plastic clay.

In the refractory trade the term "flint" clay is used to describe a hard, rocklike material which, when ground and mixed with water possesses low bonding properties. The term "plastic", "soft", or "bonding" clay is taken to mean a clay which, when ground and mixed with water, has high bonding 70 properties. The term "grog" is taken to mean "fire" clay, which has been burned at a high temperature and ground.

In addition to the fact that it serves as a satisfactory heat insulator, a hot top made 75 of this composition has higher refractory qualities and greater toughness than where plastic clay is the sole ingredient. Hot tops made of such composition do not in general suffer deterioration from breakage in shipping, or from spalling of the hot top before 80 or during a pouring operation.

In practice hot tops made of plastic clay frequently crack in all directions, in such manner as to form a net work of cracks running into each other. Hot tops made of slag frequently crumble, or else fuse under the hot temperature of the molten metal. In either case some of the material of the hot top is included in the ingot, and may work down- 105 110

wardly through the plastic metal of the ingot to a point below the sink head. This obviously has a highly deleterious effect on the metallic composition of the ingot.

5 When a hot top formed of the composition described herein does crack, such cracking is along a few well defined vertical lines, so that there is no danger that portions of the hot top may break off and be included in the metal of 10 the ingot.

Hot tops so constructed do not fuse under the temperatures attendant upon teeming an ingot, and consequently none of the material of the hot top flows and is mixed with the 15 metal of the ingot.

The composition of the present invention

may also be used for the plugs used to close the openings in ingot molds which receive the stripping plugs.

What I claim is:

1. A composition for ingot mold hot tops and plugs comprising flint clay in the relative proportion of forty per cent to sixty per cent, grog in the relative proportion of ten per cent to twenty per cent, and plastic clay. 25

2. A composition for ingot mold hot tops and plugs comprising flint clay in the approximate proportion of forty-five per cent, grog in the approximate proportion of ten per cent, and plastic clay. 30

In witness whereof, I hereunto set my hand.

EUGENE L. MESSLER.